

## UNITED STATES PATENT OFFICE

2,109,746

## HIGH SPEED ALLOY STEEL

Alvin J. Herzig, Detroit, Mich., assignor to Climax  
Molybdenum Company, a corporation of Delaware

No Drawing. Application September 12, 1935,  
Serial No. 40,254

## 8 Claims. (Cl. 75—125)

This invention relates to alloy steels and particularly those types thereof commonly known as high speed steels employed in the manufacture of cutting tools and wearing parts where 5 extreme high surface hardness is required, and particularly to such steels which include molybdenum as an alloying element thereof, the principal object being the provision of a molybdenum containing high speed steel which is particularly 10 resistant to decarburization of the surface thereof during the manufacture of the steel and the fabrication of tools and wearing parts therefrom when the steel is necessarily subjected to elevated temperatures as in forging, rolling, hardening, 15 drawing, etc.

As is well known to those skilled in the art, many steel alloys, commonly referred to as steels, are subject to the phenomenon of decarburization, rendering them unfit for service in many 20 applications. This is especially true of those steels which are used in the manufacture of cutting tools and wearing parts where extremely high surface hardness is required, which hardness cannot be obtained if carbon is lost from the 25 surface of the tool by decarburization even to the small extent of such depth as fractions of a thousandth of an inch.

A steel is said to decarburize when, by reason 30 of the conditions to which it is subjected, a lowering of the carbon content on the surface takes place. This lowering of the carbon content on the surface is accompanied by a change in the micro-structure which, in the case of many important tool steels, results in a soft skin.

35 The rate of decarburization depends upon the rate at which carbon is oxidized at the surface zone and the rapidity with which the underlying carbon diffuses into the surface oxidization zone. It has been suggested in the prior art to overcome 40 this phenomenon of decarburization by protecting the steel, when at elevated temperatures, from decarburizing atmospheres by means of coatings. These coatings may consist of electro-deposited metal or may be formed by dipping

45 the steel into molten salts or solutions of salt. It has also been suggested that the phenomenon of decarburization may be overcome by controlling the composition of the atmosphere to which the steel is subjected at elevated temperatures. 50 All of these methods afford a certain amount of protection but possess many objections either by way of being prohibitively costly, incompletely protective, or hazardous in commercial practice. For example, the use of controlled atmospheres 55 cannot be economically applied to prevent decar-

burization during forging or rolling. Electro-deposited coatings cannot always be conveniently employed by reason of the expense of equipment involved, in a great many places where tool steels are treated. The use of solutions of salt or molten 5 salt, while effective in the forging operation as well as in the heat treating operation, bring about an undesirably messy condition in the heating furnace and considerably complicates the commercial handling of the steels through the fabricating processes. 10

As is also well known to those familiar with the art, the presence of molybdenum in high speed steels, by virtue of its inherent characteristics when alloyed with iron, promotes the rate 15 of diffusion of carbon when the steels are subjected to elevated temperatures. It has been universally observed that molybdenum containing high speed steels are particularly subject to the phenomenon of decarburization and this objection alone prevents the universal use of compositions which otherwise are superior from the standpoint of cost and performance to compositions now widely used. Accompanying this decarburization it has been noted that molybdenum 20 containing steels when subjected to elevated temperatures for forging, rolling, or heat treating operations emits copious white fumes which are molybdc oxide. This invention not only prevents 25 decarburization of such steels at elevated temperatures but eliminates or materially reduces the loss of molybdenum in the surface layer through emission of this molybdc oxide. 30

This invention, therefore, relates to the discovery of alloy additions to high speed steels containing molybdenum, which additions overcome 35 the effect of molybdenum in promoting decarburization. By the use of these alloy additions molybdenum containing high speed steels may be subjected to elevated temperatures without protection against oxidizing atmosphere such as 40 ordinarily occur in furnaces, without loss of carbon from the surface and without formation of a soft skin.

More specifically, it has been found that the 45 addition of copper in amounts of 1.5% to 5% to a high speed steel containing molybdenum, markedly retards the rate of diffusion of carbon and makes it possible to expose the high speed steel containing molybdenum and copper 50 to oxid'zing atmospheres at elevated temperatures without suffering decarburization and without the formation of the so-called "soft skin." Furthermore, it has been found that the addition of copper in the above amounts may be 55

made without sacrificing the cutting properties prevalent in high speed steel containing molybdenum but not containing copper.

The high speed steel of the present invention 5 may be substantially that disclosed in United States Patent No. 1,937,334 issued November 28, 1933 to Joseph V. Emmons on Steel alloy and articles made therefrom, with the addition of copper and, if desired, other elements thereto. 10 Additionally, as will hereinafter be pointed out, substitution of the molybdenum element in the steel covered by the above patent may be made in whole or part by tungsten, within the spirit of the present invention. As an example of the 15 present invention the steel of the following composition has been found satisfactory.

|                              | Per cent  |
|------------------------------|-----------|
| Carbon                       | 0.80      |
| Manganese                    | 0.50      |
| 20 Silicon                   | 0.30      |
| Chromium                     | 4.00      |
| Molybdenum                   | 8.50      |
| Vanadium                     | 1.00      |
| Copper                       | 3.00      |
| 25 Iron and usual impurities | Remainder |

These elements may vary in percentages according to the following limits depending upon the particular characteristics desired.

|                           | Per cent      |
|---------------------------|---------------|
| 30 Carbon                 | 0.50 to 1.30  |
| Manganese                 | 0.30 to 0.80  |
| Silicon                   | 0.10 to 0.75  |
| Chromium                  | 0.20 to 10.00 |
| Molybdenum                | 0.60 to 15.00 |
| 35 Vanadium               | 0.20 to 3.00  |
| Copper                    | 1.50 to 5.00  |
| Iron and usual impurities | Remainder     |

It has also been found that .02% to .50% of 40 boron may be added to the above disclosed composition with more or less satisfactory results. 0.20% of boron gives very satisfactory results. Likewise 0.20% to 2.00% of titanium may be added to the above described composition with 45 more or less beneficial results and 0.50% is quite satisfactory. In addition tungsten may be added to the above disclosed composition with certain beneficial results. 2.00% tungsten has been found quite satisfactory. Either one, two or all 50 three of the last mentioned elements may be added in the amounts stated, if desired. Ordinarily it will be found that tungsten will have about the same final result as the molybdenum but that approximately twice as much tungsten 55 is required as molybdenum to obtain the desired results. In other words, if a particular composition of the steel described contained 1% of molybdenum and it was desired to entirely replace it by tungsten, 2% of tungsten would be required 60 to obtain the same effect as the molybdenum. Tungsten does not have the effect of promoting as rapid diffusing of the carbon in the steel as molybdenum, but the addition of copper to high speed steels of approximately the above disclosed 65 composition, except that tungsten is employed to replace the molybdenum in part or in whole, is found to be extremely beneficial. Accordingly, in the broader aspects of the present invention it will be understood that tungsten may be employed to replace either part or all of the molybdenum content set forth, so much of the molybdenum which is replaced by the tungsten being replaced by double the amount which the molybdenum content is reduced from that set forth.

It has been found that steels of the above disclosed compositions will not develop the soft skin or bark while being heated for forging and during the forging operation, that it will not decarburize during the heating operation for hardening or during hardening, and that its properties as a cutting tool are equal to, or better than, a steel of similar composition but not containing copper. It has also been found that this steel forges more readily and with less danger of cracking than a steel of similar composition but not containing copper.

It will be understood that it is within the province of the present invention to add to the above described composition elements whose additions thereto will result in well understood and expected results, and in proportions commensurate with the degree of modification desired thereby and, accordingly, it will be understood that formal changes may be made in the specific composition herein set forth without departing from the spirit or substance of the broad invention, the scope of which is commensurate with the appended claims.

What I claim is:

1. An alloy steel containing the following elements: carbon about 0.50% to 1.30%, manganese about 0.30% to 0.80%, silicon about 0.10% to 0.75%, chromium about 0.20% to 10.00%, molybdenum about 6.00% to 15.00%, vanadium about 0.20% to 3.00% and copper about 1.50% to 5.00%, said steel having high speed properties and being characterized by its resistance to surface decarburization at forging and rolling temperatures in ordinary atmospheres.

2. An alloy steel containing the following elements: carbon about 0.50% to 1.30%, manganese about 0.30% to 0.80%, silicon about 0.10% to 0.75%, chromium about 0.20% to 10.00%, molybdenum about 6.00% to 15.00%, vanadium about 0.20% to 3.00%, boron about 0.02% to 0.50%, and copper about 1.50% to 5.00%, said steel having high speed properties and being characterized by its resistance to surface decarburization at forging and rolling temperatures in ordinary atmosphere.

3. An alloy steel containing the following elements: carbon about 0.50% to 1.30%, manganese about 0.30% to 0.80%, silicon about 0.10% to 0.75%, chromium about 0.20% to 10.00%, molybdenum about 6.00% to 15.00%, vanadium about 0.20% to 3.00%, tungsten about 2.00%, and copper about 1.50% to 5.00%, said steel having high speed properties and being characterized by its resistance to surface decarburization at forging and rolling temperatures in ordinary atmospheres.

4. An alloy steel containing the following elements: carbon about 0.50% to 1.30%, manganese about 0.30% to 0.80%, silicon about 0.10% to 0.75%, chromium about 0.20% to 10.00%, molybdenum about 6.00% to 15.00%, vanadium about 0.20% to 3.00%, boron about 0.02% to 0.50%, tungsten about 2.00%, and copper about 1.50% to 5.00%, said steel having high speed properties and being characterized by its resistance to surface decarburization at forging and rolling temperatures in ordinary atmospheres.

5. An alloy steel comprising the following elements: carbon about 0.80%, manganese about 0.50%, silicon about 0.30%, chromium about 4.00%, molybdenum about 8.50%, vanadium about 1.00%, and copper about 3.00%; said steel being characterized by having high speed properties and by being resistant to surface decar-

burization at forging and rolling temperatures in ordinary atmosphere.

6. An alloy steel comprising the following elements: carbon about 0.80%, manganese about 0.50%, silicon about 0.30%, chromium about 4.00%, molybdenum about 8.50%, vanadium about 1.00%, boron about 0.20% and copper about 3.00%; said steel being characterized by having high speed properties and by being resistant to surface decarburization at forging and rolling temperatures in ordinary atmospheres.
10. An alloy steel comprising the following elements: carbon about 0.80%, manganese about 0.50%, silicon about 0.30%, chromium about 4.00%, molybdenum about 8.50%, vanadium
15. An alloy steel comprising the following elements: carbon about 0.80%, manganese about 0.50%, silicon about 0.30%, chromium about 4.00%, molybdenum about 8.50%, vanadium

about 1.00%, boron about 0.20%, tungsten about 2.00%, and copper about 3.00%; said steel being characterized by having high speed properties and by being resistant to surface decarburization at forging and rolling temperatures in ordinary atmospheres.

8. An alloy steel comprising the following essential elements: carbon about 0.50% to 0.85%, chromium about 4.00%, molybdenum about 8.50%, copper about 3.00%, and boron 0.03% to 0.50%, said steel having high speed properties and being characterized by its resistance to surface decarburization at forging and heat treating temperatures in ordinary atmospheres.

ALVIN J. HERZIG. 15